

June 12, 1934.

S. D. WELLS

1,962,164

METHOD AND APPARATUS FOR REMOVING PRINTING INK FROM PAPER

Filed Sept. 6, 1932



## UNITED STATES PATENT OFFICE

1,962,164

METHOD AND APPARATUS FOR REMOVING  
PRINTING INK FROM PAPERSidney D. Wells, Appleton, Wis., assignor to  
Lewis L. Alsted, Appleton, Wis.

Application September 6, 1932, Serial No. 631,805

18 Claims. (Cl. 92—11)

This invention relates to a method of and apparatus for removing printing ink from paper and is particularly adapted for use in recovering old paper stock containing mechanical wood pulp and which has been printed upon with a special type of ink, as, for example, an ink of the type disclosed in the pending application of Alex B. Davis, James F. Thompson and Alfred T. Gardner for a Process for the recovery of pulp from printed paper, filed October 24, 1931, Serial No. 570,968 and assigned to Lewis L. Alsted of Appleton, Wisconsin, the assignee of this application.

Certain sources of supply of old paper stock such as newspapers, directories and particularly telephone directories, books, catalogues and the like, become after a certain length of time obsolete and are replaced by current issues, so that such material may be conveniently collected to provide an available source of supply of stock for repulping into paper. However, even where such material is printed with a special type of ink, readily converted into colorless substances or substances corresponding in color to that of the original color of the pulp, the stock, when pulped, and as heretofore treated, so retards the passage of water or other fluid through it as to present a serious and difficult problem insofar as removal of the ink or other undesirable matter is concerned.

One of the objects of the present invention is to provide a method of and an apparatus for removing printing ink and other impurities or undesirable matter from old paper stock which is susceptible of practice on a commercial scale and with economies consistent with the requirements of actual commercial activity, and which so conditions and treats the stock as to subject all of the fibers thereof to the action of the de-inking and cleansing medium in an efficient and effective manner whereby to completely de-ink the old stock and convert it into a pulp possessed of all of the desirable characteristics of unused pulp and suitable for manufacture into paper having the color, texture, strength and other desirable qualities which the paper of the old stock originally possessed.

Broadly, the present invention consists in first beating the old paper stock under such conditions and to such extent as to nodulize the stock, that is, to work the same up into small pellets of uniform size, with each pellet containing a relatively great amount of water and a small amount of fiber. A batch of such nodulized stock is then subjected to the action of a

de-inking and cleansing medium in such manner that the de-inking medium permeates all of the fibers of the pellets under the influence of diffusion to dissolve the ingredients of the ink and other impurities and carry them off in solution with the de-inking medium. A washing medium is then employed and also exerts its action under the influence of diffusion and as a result the pellets, after such treatment, are free of ink or other impurities and consists entirely of fiber and water, the latter being slightly acidulated, if desired.

An important feature of the invention resides in effecting the de-inking or cleansing by diffusion. This is especially advantageous with the nodulized stock since the de-inking, by sulphurous acid, for example, is effected without breaking down the nodules, whereby any tendency of the fibers to mat and retard the cleansing or de-inking action is precluded. Furthermore, with a diffusion treatment, the stock retains its nodulized characteristics throughout the various stages of a multistage treatment and during its final washing.

More specifically, the present invention contemplates the reduction of the waste paper to nodules or pellets in a rod mill, or in a pulper or kneader, or in a combination of a beater and de-watering device (such as a screw press). The nodulized stock is then transferred to diffusers, preferably in the form of closed tanks, wherein the nodules are subjected to the action of sulphur dioxide which is converted into sulphurous acid when diffused through and combined with the water in the nodules. In lieu of the use of sulphur dioxide a solution of sulphurous acid may be employed and preferably the treatment is carried out by using alternately weak and strong solutions of sulphurous acid. Sulphurous acid is desirable since it also acts as a reducing agent to discharge the ink and render it soluble in the dilute acid. Where inks are encountered which are soluble in an acid without necessitating any reduction, acids other than sulphurous acid may be employed, for example, sulphuric acid. However, since sulphurous acid combines acidity with reducing properties, it is usually preferable. The acid utilized is caused to travel through the diffusers and during its passage, is diffused throughout the nodules, to discharge the ink and dissolve it and thereby carry it off in solution. Following this treatment water is passed through the diffusers to effect appropriate washing and removal of sulphurous acid. In some instances, in order to stabilize the results obtained and counteract

80

85

90

95

100

105

110

any conflicting tendencies or deleterious effects that may arise from local water conditions or for other reasons it may be desirable to use water acidulated with sulphuric acid or some other 5 equivalent strong acidulating agent. After such treatment the nodules are transferred to a stuff chest wherein the stirring action of the agitators readily resolve the nodules into a pulp possessing the appearance and the characteristics of unused 10 pulp appropriate for manufacture into paper.

In the drawing;

The figure is a diagrammatic representation of one type of apparatus appropriate for carrying out the method of the present invention.

15 As shown in the drawing, the old paper stock is fed in any suitable way, as by means of a conveyor 1, into a rod mill designated generally at 2 which is of conventional construction in that it has the ordinary drum 3 rotated by power driven 20 gearing 4 and containing a number of loose rods (not shown) extending longitudinally thereof and parallel to each other in the usual manner. For a full disclosure of such a rod mill, reference is made to my application for Apparatus and method 25 of removing printing ink from paper, filed June 29, 1932, Serial No. 619,983. In the rod mill the old stock is subjected to the beating and rubbing action of the rods which disintegrates the paper and reduces it to fibers, without, however, injur- 30 ing the fibers. As this beating and rubbing action is carried on in a water solution at relatively high consistencies, nodulization of the paper stock is effected, that is to say, with a small amount of water, the rubbing action on the stock is such as 35 to work the fibers and the other ingredients of the disintegrated stock into pellets or nodules of uniform size and of high moisture content. The nodules so formed are substantially one-sixteenth to one-eighth inch diameter and possess a free- 40 ness on the Canadian freeness tester of from 600 to 700 as compared to a freeness of 140 possessed by similar stock pulped in the ordinary way. The consistencies which may be advantageously employed range from approximately 12% to about 45 33%. The consistency usually employed is in the neighborhood of twenty five per cent, that is, three parts of water to one part of fiber.

The nodulized stock is transferred from the rod mill to one or more diffusers of which two, designated at 5 and 6, are illustrated. For the purpose of simplicity in illustration, the transferring is shown as being effected through a pipe 7 leading into the diffuser 6 and having a branch 8 leading 55 into the diffuser 5. Gates or valves 10 and 11 are provided to regulate or shut off the flow through the pipes 7 and 8 and a suitably operated screw conveyor 13 may be provided for advancing the nodules through a portion at least of the pipe 8.

60 The diffusers are of similar construction and each includes a closed tank 15, each tank having a cylindrical body portion provided with a closed top 16 and a closed bottom 17. Within each tank a perforated false bottom 18 and a perforated false top 19 is provided, the false bottom 18 and the false top 19 being spaced from the bottom 17 and the top 19, respectively. The pipes 7 and 8 lead through the tops 16 and also through a suitable opening provided in the false top 19 so as to discharge into 65 the space between the false bottom and top of each tank. At a convenient point, a storage tank 20 for sulphur dioxide is provided and connects by means of a pipe 21 and branches 22 and 23 with the tanks 5 and 6, respectively. A valve 24 70 is provided in the pipe line 21 and similar valves 75

25 and 26 are provided in the branches 22 and 23 whereby the supply of gas from the tank 20 may be shut off adjacent the tank or may be shut off adjacent either diffuser. The valves 24, 25 and 26 may be manipulated to supply sulphur dioxide to either or both diffusers. More than two diffusers may be employed, if desired.

Tanks 30 and 31 are provided for containing sulphurous acid gas, the tank 30 for strong solution of sulphurous acid and the tank 31 for a weaker solution. The bottoms of the tanks 30 and 31 are connected by valve controlled pipes 32 and 33 to a pipe line 34 leading to a pump 35 which delivers to a pipe line 36 having valve control branches 37 and 38 leading into the diffusers 5 and 6. The pipes which supply sulphur dioxide or sulphurous acid to the diffusers lead through the bottoms thereof so that they discharge into the space between the bottom 17 and the false bottom 18 of each diffuser. The upper ends of the tanks connect with branches 40 and 41 equipped with valves 42 and 43 and communicating with a return pipe line 44 having valve control branches 45 and 46 which lead into the tanks 30 and 31, respectively. The pipe line 44 is extended, as indicated at 47, to a point of suitable discharge or to suitable recovery apparatus (not shown), and its communication with the discharge or recovery apparatus connection is controlled by a valve 49. The recovery apparatus 90 may consist of a suitable combination of heat interchanger and evaporator effective to recover sulphur dioxide from the used acid solution and, if desired, of suitable means for facilitating recovery of the ink by coagulation and filtration.

100 The diffuser tanks 5 and 6 are provided with suitable valve controlled outlet connections designated at 50 and 51 and with suitable manhole openings 52 and 53. The outlet connections 50 and 51 discharge into a stuff chest 55 provided 105 with a stirrer or agitator designated at 56.

110 In the rod mill the paper stock is completely de-fibered and the ink and other impurities loosened and the stock is worked up into pellets or nodules containing a relatively large amount of water, 115 for example, from about six times to three times the weight of water to the weight of pulp. This, however, may vary and where, under the necessity of considerable handling, there is the requirement that the nodule characteristics be retained, the water content usually should be kept within four times that of the fiber, that is, 20% pulp to 80% moisture.

120 The nodules are then transferred to the diffusers 5 and 6 where both diffusers are used and in the first instances the valves 24, 25 and 26 are open so that sulphur dioxide is admitted to the interior of the diffusers and combines with the water in the nodules to form sulphurous acid. After this treatment the valves 24, 25 and 26 are 125 closed and the valve controlled branch 32 from the strong liquor tank 30 is opened so that strong liquor or a strong solution of sulphurous acid may be pumped by the pump 35 through the pipe line 36 and through the valve control branches 37 and 38 thereof into the lower ends of the diffusers. 130 This strong solution of sulphurous acid is usually derived, in actual practice, from the leaching of a previous batch and consists of a solution of sulphurous acid with some ink dissolved therein. The approximate concentration of this strong 135 solution is about 1.8% sulphur dioxide. As the strong solution travels up through the diffuser it is diffused through the nodules and therein it takes more ink and its concentration tends to 140 145 150

vary, it becoming stronger at the bottom of the diffuser where the nodules are more strongly impregnated with sulphurous acid and weaker at the top where the nodules contain less sulphurous acid. As the treatment goes on, however, this variation becomes less and less and a uniform concentration and impregnation occurs. The liquid during its passage through the diffuser surrounds the nodules and is immediately absorbed therein due to their capillary attraction. In this way any substances in the ink capable of reduction are reduced; the ingredients of the ink are rendered soluble; and the sulphurous acid provides a solvent for such ink ingredients.

15 Depending upon its condition, which is observed or tested when leaving the diffusers, the strong liquor is either carried back to the strong liquor tank, or the weak liquor tank, or else is carried to a point of discharge or to suitable apparatus for recovering the sulphur dioxide and ink therefrom.

20 When the concentration in the diffuser is entirely uniform the supply of strong liquor is cut off and weak liquor is supplied to the diffuser or diffusers from the weak liquor tank 31 by closing the valve 32 and opening the valve 33. The weak liquor may have a concentration of .5% sulphur dioxide. The weak liquor is put through the diffusers, for the purpose of picking up all 25 of the sulphurous acid that can be received from the nodules and depending on its condition is carried back from the diffusers to the strong liquor tank 30 or weak liquor tank 31 for reuse or else is taken to the recovery apparatus when 30 the sulphur dioxide and also the ink, if desired, is reclaimed. Dissolved ingredients of the ink or other dissolved impurities are, of course, carried off with the weak liquor.

35 After sufficient weak liquor has been supplied to each diffuser to create a definite zone the weak liquor is shut off by closing the valve 33 and water is supplied to the lower ends of the diffusers and travels upwardly therefrom to wash out any remaining sulphurous acid together with any remaining ink dissolved therein. The rate at 40 which the liquor is passed through the diffuser is sufficiently fast to preclude any material downward diffusion, that is, dilution of the zone above by the zone below. The depth of zone, however, should be great enough so that by the time a definite zone has passed any strata complete equalization (of strength or concentration) of the liquor around and in the nodules has taken place; or, in the washing operation, effective washing 45 consummated.

50 By having the final washing carried out with acidulated water, any traces of the ingredients of the ink remaining in the fibers are converted to chemically stable compounds and in general the results obtained are stabilized and any deleterious effects arising from the use of the water employed or otherwise are counteracted.

55 After the nodulized stock has been treated in the manner described in the diffusers 5 and 6, the outlets 50 and 51 are open and the stock dumped or flushed into the stuff chest 55. If desired, a hose may be inserted through the manholes 52 and 53 and utilized to flush out the treated stock. In the stuff chest the nodulized stock is broken up or resolved into pulp and may be readily manufactured into paper.

60 It is to be understood that the present invention, in its broader aspects, is not limited to a de-inkable ink of any particular composition or to any specific de-inking medium. The main ad-

vantages of the present invention are realized by nodulizing the stock and subjecting it to a diffusion treatment with a de-inking or cleansing medium, whatever may be the composition of the de-inkable ink or the character of the de-inking medium. Within a corresponding range, the subsidiary advantage of stabilizing the results obtained are had by a final washing with an acidulated medium. In its more specific aspects, the present invention consists in the utilization, in the diffusion treatment and in the novel manner set forth of sulphur dioxide or of sulphurous acid as the de-inking medium.

65 It is also understood that the process can be applied to the removal from paper of coloring matter, which is dischargeable or soluble in suitable solution of acids, alkalis or salts, or in water alone.

70 The apparatus and method specifically described have been selected for purposes of illustration and example and various changes in form, sequence, reagents, and proportions, as well as various omissions or additions may be resorted to without departing from the spirit of the invention or the scope of the subjoined 75 claims.

The invention claimed is:

1. The herein described method of de-inking printed paper which comprises nodulizing the paper, subjecting the nodulized stock to an upwardly traveling bath of de-inking fluid so that the de-inking fluid permeates the nodulized stock by diffusion to discharge the ink therefrom and then subjecting the stock to a diffusion washing to remove the de-inking fluid with the ink ingredients from the stock.

105 2. The herein described method of de-inking printed paper which comprises nodulizing the paper, subjecting the nodulized stock to an upwardly traveling bath of de-inking fluid so that the de-inking fluid permeates the nodulized stock by diffusion.

110 3. The herein described method of de-inking printed paper which comprises nodulizing the paper, subjecting the nodulized stock to a diffusion treatment with a fluid de-inking medium.

115 4. The herein described method of de-inking printed paper which comprises nodulizing the paper, subjecting the nodulized stock to a diffusion treatment with sulphurous acid.

120 5. The herein described method of removing printing ink from paper which comprises subjecting the paper to a beating and rubbing action in water and at a high consistency until the paper is reduced to fibers and worked up into nodules having a high water content, and then subjecting the nodulized stock to a diffusion treatment with sulphur dioxide whereby sulphurous acid is formed in the nodules to provide a reducing agent and a solvent for the ingredients of the ink.

125 6. The herein described method of removing printing ink from paper which comprises subjecting the paper to a beating and rubbing action in water and at a high consistency until the paper is reduced to fibers and worked up into nodules having a high water content, and then subjecting the nodulized stock to a diffusion treatment with sulphurous acid.

130 7. The herein described method of removing printing ink from paper which comprises subjecting the paper to a beating and rubbing action in water and at a high consistency until the paper is reduced to fibers and worked up into nodules having a high water content, then subjecting the 135

140

145

nodulized stock to a diffusion treatment with sulphur dioxide whereby sulphurous acid is formed in the nodules to provide a reducing agent and a solvent for the ingredients of the ink, and then 5 subjecting the stock to a diffusion washing.

8. The herein described method of removing printing ink from paper which comprises subjecting the paper to a beating and rubbing action in water and at a high consistency until the paper 10 is reduced to fibers and worked up into nodules having a high water content, then subjecting the nodulized stock to a diffusion treatment with sulphur dioxide whereby sulphurous acid is formed in the nodules to provide a reducing agent and a 15 solvent for the ingredients of the ink, and then subjecting the stock to a diffusion washing with acidulated water.

9. The herein described method of reclaiming old paper stock which comprises nodulizing the 20 stock and thereafter subjecting it to a diffusion treatment with a cleansing fluid.

10. The herein described method of reclaiming old paper stock which comprises nodulizing the 25 stock and subjecting the nodulized stock to a diffusion treatment with sulphurous acid.

11. The herein described method of reclaiming old paper stock which comprises beating the 30 stock in the presence of water and at high consistencies until the stock is reduced to fibers and worked up into pellets and thereafter subjecting the stock to a diffusion treatment with a fluid ink 35 removing medium.

12. The herein described method of reclaiming old paper stock containing mechanical ground 35 wood pulp which comprises beating the stock in a solution at high consistencies and until the stock is nodulized and thereafter subjecting the stock to a diffusion treatment with sulphurous acid and finally to a washing operation with acidulated water.

13. The herein described method of reclaiming old paper stock containing mechanical ground 40 wood pulp which comprises beating the stock in a solution at high consistencies and until the stock is nodulized and thereafter subjecting the stock to a diffusion treatment with sulphurous acid.

14. An apparatus for de-inking paper comprising means for disintegrating the paper into fibers in a water solution and nodulizing the fibers, a 45 diffuser for receiving and containing the nodulized stock, and a circulation system for subjecting the nodulized stock in the diffuser to an upwardly traveling bath of sulphurous acid whereby the sulphurous acid permeates the nodules by diffusion and thereby discharges the ink therefrom.

15. An apparatus for de-inking paper, compris-

ing means for disintegrating the paper into fibers in a water solution and nodulizing the fibers, a diffuser for receiving and containing the nodulized stock, and a circulation system including tanks containing strong and weak solutions of sulphurous acid, valve controlled supply and return connections between said tanks and said diffuser and a pump in said supply connection whereby the nodulized stock in the diffuser may be subjected to successive baths with strong and weak sulphurous acid in such manner that the 80 said permeates the nodules by diffusion and thereby discharges the ink therefrom.

16. An apparatus for de-inking paper comprising means for disintegrating the paper into fibers in a water solution and nodulizing the fibers, a diffuser for receiving and containing the nodulized stock, and a circulation system including tanks containing strong and weak solutions of sulphurous acid, valve controlled supply and return connections between said tanks and said diffuser and a pump in said supply connection whereby the nodulized stock in the diffuser may be subjected to successive baths with strong and weak sulphurous acid in such manner that the 85 said permeates the nodules by diffusion and thereby discharges the ink therefrom. 90

95

100

105

110

115

120

125

130

SIDNEY D. WELLS. 130